

Oct. 29, 1935.

F. ROTHER

2,019,096

PRODUCTION OF SUPPRESSION LAYER PHOTOCELLS

Filed July 7, 1933

Fig. 1



Fig. 2



By

Inventor:  
Franz Rother  
Bolley & Hinman  
Attorney

## UNITED STATES PATENT OFFICE

2,019,096

PRODUCTION OF SUPPRESSION LAYER  
PHOTOCELLS

Franz Rother, Paris, France

Application July 7, 1933, Serial No. 679,285  
In Germany July 8, 1932

6 Claims. (Cl. 136—89)

This invention relates to improvements in suppression layer cathodes for photo cells and the like and to a method for manufacturing the same.

An object of the invention is to provide a cell 5 of the aforementioned character having improved sensitivity and efficiency.

Another object is to provide a cell of great durability.

Another object is to provide a cell which can 10 be easily manufactured.

Another object is to provide a method for manufacturing a cell of the aforementioned character.

Other objects and advantages will hereinafter 15 appear.

An embodiment of my invention will be explained in the following description with reference to the appended drawing in which

Figure 1 is a cross sectional view of the construction of a cell as used heretofore, while

Fig. 2 is a similar view of a cell constructed in accordance with my invention.

The suppression layer photo-cells were hitherto produced, for example in the case of the copper-cuprous oxide cell, by heating a metallic copper plate to about 1020° C. for some time in a furnace in the presence of oxygen.

The known suppression layer photo-cell is illustrated diagrammatically in section in Fig. 1. 30 The cell removed from the furnace shows on its surface copper oxide which is removed by suitable processes, so that the cuprous oxide layer 3 is exposed which is located under the copper oxide and has grown on the mother copper 1. The very thin hypothetic "suppression layer" 2 which is permeable for the electrons only in one direction, is situated between the cuprous oxide layer 3 and the metallic copper support (mother copper) 1. The mother copper plate 1 serves as one of 35 the electrodes of the finished suppression layer cell, whereas usually a thin metal layer 4 applied on the cuprous oxide layer 3 by known processes, such as cathode atomizing, serves as second or counter electrode.

40 It has now been found that the photo-electric effect of such suppression layer photo cells can be considerably increased if the metallic copper plate 1, in the case of a copper-cuprous-oxide cell, is coated with a layer 5 of another metal as shown in Fig. 2 before being brought to a high temperature. The coating 5 may be applied to the mother copper plate 1 by cathode atomizing, electrolysis, by a spraying process or by any other suitable process. If, for example, a copper plate 45 50 55 1 is coated with a gold layer 5 before being

brought to a high temperature, this gold layer 5 remains on the copper after the finishing of the cell or is partly alloyed with the latter at its surface and the cuprous-oxide layer 3 has formed over the gold layer 5. Consequently over the mother copper 1 there is besides the known thin suppression layer 2 also the gold or gold alloy layer 5 and above this the cuprous oxide layer. Such a suppression layer photo-cell, however, as compared with a similar cell but without the gold 10 layer 5 previously applied onto the copper 1, shows about 10 times greater photo-electric effect or a ten times greater energy yield under otherwise similar conditions.

The metal layer 5, applied to the metallic copper 1, may be extremely thin, so thin that it is translucent. Such a cell also presents the advantage over the known cells as regards production, that the cuprous oxide 3 uniformly covers the whole surface of the cell and chipping off of a 20 portion of the cuprous oxide layer when removing the cell from the furnace or during the cooling, as often happens in the production of the known cells, being avoided. The copper plate 1, in the case of copper-cuprous oxide cells, may also be 25 covered with two or more thin, superposed metal layers 5 before it is brought to a high temperature.

35 By this process other metals besides copper may be employed as mother metal 1 for producing suppression layer photo cells. The copper 1 under the applied gold layer 5 diffuses into and through the thin gold layer at the production temperature of the cell, so that the oxygen compounds of the copper then form on the gold or 35 gold alloy layer 5.

The new process is particularly practical if the mother metal, on which the thin metal coating 5 is applied, is not a pure metal but a metal alloy which may consist of two or more components. 40 Precious metals are particularly suitable as coating metal 5 in the sense of the invention, but any of the metals may be employed except the metals of the alkali group. If, however, more than one coating layer 5 is to be employed, thin 45 layers of metals which can easily oxidize, may be applied over or under the precious metal layer. Fig. 2 must be regarded merely as a diagrammatic view.

I claim:

50 1. In the process of producing suppression layer cathodes for photo cells and the like, comprising a copper base and a coating of an oxide thereof, the step which consists in coating said base with a thin layer of another metal not 55

belonging to the alkali group of metals and thereafter heating the so coated base to thereby cause copper to diffuse into and to form an alloy with said other metal and further to oxidize at least 5 part of the copper so diffused to form said oxide coating overlying said alloy.

2. In the process of producing suppression layer cathodes for photo cells and the like, comprising a copper base and a coating of an oxide thereof, the step which consists in coating said base with a thin layer of a precious metal and thereafter heating the so coated base to thereby cause copper to diffuse into and to form an alloy with said precious metal and further to oxidize 10 at least some of the copper so diffused to form an oxide of said copper overlying the surface of said alloy.

3. In the process of producing suppression layer cathodes for photo cells and the like, comprising a copper base and a coating of an oxide thereof, the step which consists in coating said base with a plurality of successive thin layers of different other metals not belonging to the alkali group of metals and thereafter heating the 15 so coated copper base to thereby cause copper to diffuse into and to form alloys with said differ-

ent other metals and further to oxidize at least some of the copper so diffused to form an oxide of said copper overlying said alloys.

4. A suppression layer photo cell comprising, in combination with a copper base and a layer of an oxide thereof, an alloy of said copper and another metal not belonging to the alkali group of metals interposed between said copper base and said layer and adhering to said copper base and said oxide by an inter-molecular bond. 10

5. A suppression layer photo cell comprising, in combination with a copper base and a layer of an oxide thereof, an alloy of said copper and a precious metal interposed between said copper base and said layer and adhering to said copper 15 base and said oxide by an inter-molecular bond.

6. A suppression layer photo cell comprising, in combination a copper base and a layer of an oxide thereof, a plurality of thin layers of alloys of different other metals not belonging to the alkali group of metals and said copper, said layers being interposed between said copper base and said oxide layer, said copper base and said layers adhering to one another at their respective boundaries by an inter-molecular bond. 20 25

FRANZ ROTHER.